

March 5, 1935.

H. KRANICH

1,993,517

ARTIFICIAL FUEL AND PROCESS OF MAKING SAME

Filed July 29, 1931



INVENTOR

*Herbert Kranich*  
BY  
*Lyman E. Dodge*  
ATTORNEY

## UNITED STATES PATENT OFFICE

1,993,517

ARTIFICIAL FUEL AND PROCESS OF  
MAKING SAME

Herbert Kranich, West Hempstead, N. Y.

Application July 29, 1931, Serial No. 553,741

5 Claims. (Cl. 44—7)

This invention relates to cellulose compounds such as cellulose nitrate and acetate, sometimes called nitro-cellulose and aceto-cellulose, and particularly to so called solutions of such cellulose compounds, and more especially to a method and means for causing what is known as, solidification of such solutions.

5

Heretofore, various kinds of cellulose compounds have been dissolved in various menstrua, and then various kinds and methods have been employed to solidify the cellulose compound whereby the menstrua will be contained in a framework of cellulose compound thereby producing what is commonly called "solid alcohol".

10

15 Methods and means heretofore used in order to obtain a satisfactory solid alcohol have either required rather complicated mechanisms, difficult to keep free from deposits of solidified cellulose compound, or have been of such a nature that the solidifying agent introduced into the solution could not be easily controlled within narrow limits.

20 A principal object of this invention is the production of a means and method for the solidification of a cellulose compound solution such that complicated and cumbersome machinery is obviated, together with the attendant difficulties due to the deposit of solidified cellulose compound upon the operative parts of the interior 25 and exterior of such machines.

25 A further object of this invention is the production of a means and method for the purpose specified which will enable a solidification to be accomplished by the introduction of a solidification agent which may be controlled as to quantity within quite narrow limits.

30 A further object of this invention is the production of a means and method for the purpose specified which will result in the production of a product quite thoroughly homogeneous and uniform throughout, thereby insuring a constant uniform burning without frequent flaring up and dying down.

35 A further object of this invention is the production of a means and method for the purpose specified which will be inexpensive, result in the least amount of waste by-product, and which may be usable successfully by persons of slight manipulative skill.

40 Other objects and advantages will appear as the description of the particular physical embodiments selected to illustrate the invention progresses, and the novel features will be particularly pointed out in the appended claims.

45 In describing the invention in detail, and the

particular physical embodiments selected to illustrate the invention, reference will be had to the accompanying drawing and the characters of reference thereon.

5 The drawing, by a single figure, illustrates a solid alcohol container with solidified material therein and a solidifying means made in accordance with my invention is placed therein.

10 In order to carry out my invention, I select a cellulose compound which is soluble in the particular solvent which I intend to use for making a solution thereof. Nitro-celluloses are obtainable which are soluble in commercial methyl alcohol.

15 The solvent power of the commercial methyl alcohol is, as is well known, due to the presence therein of acetone. Nitro-cellulose of a nitrogen content may be obtained which are soluble in anhydrous ethyl alcohol. When a nitro-cellulose which is soluble in anhydrous ethyl alcohol is used, the nitro-cellulose after being dissolved in a small quantity of anhydrous ethyl alcohol may then be diluted largely with an ordinary ethyl alcohol, which may contain from 5 to 10% of water, without coagulating or precipitating the dissolved nitro-cellulose. The diluting alcohol may contain in addition to water, a denaturant, such as methyl alcohol or pyridine, without causing a precipitation of the dissolved nitro-cellulose. I may use a nitro-cellulose soluble in amyl acetate and after the solution of nitro-cellulose dilute with ordinary ethyl alcohol in the same manner as, above described, in a case of nitro-cellulose soluble in anhydrous ethyl alcohol.

20

25 I may also form a nitro-cellulose solution quite comparable with the ordinary collodion of commerce, that is, I may dissolve a nitro-cellulose in any alcohol-ether mixture. The ether ordinarily used in making ordinary pharmaceutical collodion is ethyl ether, but I may substitute for that ether, another ether, such as methyl ether, or propyl ether, or use a mixed or compound ether, such as methyl-ethyl, or ethyl-propyl ether.

30

35 In fact there are an innumerable number of nitro-cellulose solvents suitable for use as solvents for a nitro-cellulose to be used, in accordance with my method, for the making of a solid alcohol. The determining characteristic of the solvent to be used resides in the fact that the nitro-cellulose must be precipitable therefrom by means of water, either as a liquid, or a solid as in the case of ice, or as a vapor as in the case of steam.

40 Instead of nitro-cellulose I may use other cellulose esters, such as cellulose acetate, or prefer-

5

10

15

20

25

30

35

40

45

50

55

ably, a hydrated sulpho-nitro-cellulose acetate, such as has been described in my copending application filed on even date herewith Serial No. 553,739. In case I use the hydrated sulpho-nitro-cellulose acetate I would prefer the form thereof soluble in cold 95% water diluted pure ethyl alcohol. Another solvent particularly applicable to the last named base would be a mixture of 95% water diluted ethyl alcohol and 95% water 10 diluted commercial methyl alcohol.

The particular solvent preferred by me, when using nitro-cellulose is anhydrous ethyl alcohol. The particular diluent preferred by me is the ordinary pure ethyl alcohol containing not over, 15 about 5% of water and containing as a denaturant if necessary, on account of governmental regulations, methyl alcohol, and preferably free from substances which produce an evil or disagreeable odor when burned, such as pyridine.

20 Various quantities of nitro-cellulose soluble in anhydrous ethyl alcohol, may be dissolved in anhydrous ethyl alcohol, but for my purposes, I prefer to dissolve approximately 3 pounds of substantially nitro-cellulose, made anhydrous by alcohol displacement, in 40 pounds of anhydrous ethyl alcohol either pure or denatured as required by governmental regulations. After complete solution, various amounts of diluents may be added thereto, but I prefer to add to such a 25 solution, as is just above described, approximately 60 pounds of about 95% ethyl alcohol, denatured by the addition of the smallest quantity possible, in compliance with governmental regulations, of methyl alcohol. Such a procedure should give 30 me a nitro-cellulose alcohol solution containing about 3% of nitro-cellulose.

Having obtained a suitable nitro-cellulose solution, it may then be run into any suitable containing vessel, so that it appears as a broad, relatively thin sheet, or as a narrow elongated prism. For my purposes, however, I prefer to run the solution of nitro-cellulose directly into containers in which it is to be dispensed. Such a container is shown in the drawing and designated 1. It is 40 of a usual form, and consists essentially of a hollow cylinder provided with a bottom portion 2, and an annulus 3 at the top thereof which is adapted and constructed to receive and tightly hold a cover which may be sprung into place and 45 securely held by the resilience of the material and which may be pried open by almost any pointed tool. The can or container 1, should not be filled up to the annulus, but a space should be left between the annulus and the top of the alcoholic solution of a cellulose ester. The reason 50 for this will appear hereinafter.

In order to solidify the alcoholic solution of nitro-cellulose a precipitant, or coagulant, or solidifying agent must be introduced into the 55 solution. This solidifying agent I prefer to introduce, in such a manner as not to disturb the homogeneity or uniformity of the solution. The solidifying agent may be poured upon the top of the solution. If water is used as a solidifying agent, as soon as the water touches the top surface of the nitro-cellulose solution, a solidification will take place and the water will remain upon the top of the solution until such time as diffusion has taken place throughout the entire 60 mass whereby the water top of the solution will be exchanged for alcohol, and perhaps solvent in the solution, until the fluid on top of the solution arrives at substantially the same percentage composition as the solution held within the frame- 70 work or pores of the nitro-cellulose which has

become solidified. This process takes a very considerable amount of time, relatively speaking, and therefore is objectionable.

The nitrocellulose solution may be solidified by what might be called an immersion method. In order to carry this out successfully, the nitro-cellulose solution may be poured upon a sheet of material impervious to the solution, such as, moistened cotton placed in the bottom of a pan having a perforated bottom, then the pan placed 10 in a body of water so that the top edge thereof is not below the surface of the water. This method may be used but its use necessitates the later cutting of the mass into small bodies adapted for being packed into a container such as 1, 15 so that an extra operation is required.

In order to obviate the difficulties of the prior methods described, and in order to obtain a uniform and homogeneous product, applicant prefers to solidify the nitro-cellulose solution in 20 the container in which it is to be dispensed, and to that end, and in accordance with his invention introduces, as manually, a somewhat elongated solidifying means 5 into the nitro-cellulose solution. This solidifying body 5 should be such 25 length that, when its lower end rests upon the bottom 2 of the can, its upper end will be at least slightly above the upper line 6 of the nitro-cellulose solution. By such proportioning, the nitro-cellulose will not form a layer over the top of the 30 body 6, and so it may be withdrawn quite readily after the solidifying action has taken place. As a further aid in withdrawing the body 5, I prefer to extend it to some little height above the nitro-cellulose solution, in order that it may be 35 grasped by thumb and fingers and withdrawn after the solidification action has taken place. Of course, I do not mean by this description to exclude other constructions which do not necessitate carrying the body 5 to the height specified, 40 and do not intend to exclude specifically such constructions as to involve a manipulating member, as a rod, imbedded in the member 5 and protruding from the top thereof which would allow the member 5 to be of less length and still 45 be capable of manual manipulation in withdrawing the same from the body of the nitro-cellulose. In any event, the top of the member 5 must be such that after the member 5 has been put in place the cover 4 may be put in place, and the can with its contents of nitro-cellulose solution and the solidifying member 5 may be set aside until such time as the solidification has taken 50 place.

As a solidifying body 5, I may use a substance 55 which is sufficiently solid to substantially retain its form and of sufficient structural strength to enable it to be manually handled, and which is characterized by its ability to contain a solidifying liquid capable of being diffused from the body to and throughout the mass of nitro-cellulose solution, and a body to which the solidified nitro-cellulose will not adhere after being solidified, so that the body may be easily withdrawn therefrom.

As a solidifying substance, I prefer the use of water and as a body to carry the water I prefer a body of soap.

The particular soap preferred by me for use 70 with my invention is one which I make by a method preferred by me. This method consists in taking stearic acid and boiling it with alcohol and water, then after adding a few drops of phenol-phthalein as an indicator, cautiously adding 75 30 degrees Baumé caustic soda solution until the

entire solution just turns red, and then allowing the mass to stand until cold. When the mass is cold it will be quite hard and firm and may be cut into any desired shaped bodies, such as prisms. Suitable proportions for making this soap are 4 grams of stearic acid, 25 grams of alcohol, 75 grams of water and sufficient of the designated caustic soda solution to neutralize the stearic acid and form sodium stearate. Such proportions would give about a 4% soap solution.

Of course, by the specific mentioned of stearic acid, I do not intend to exclude other well known fatty acids which are well known equivalents of stearic acid.

In order to properly effectuate the solidification which I desire, I take a plug weighing approximately from 15 to 18 grams made of the solid soap above described, to about 100 cubic centimeters of nitro-cellulose solution, that is, the plug 5 would be adjusted in size to correspond, in accordance with the given proportions, with the quantity of nitro-cellulose solution in the container 1.

I prefer to allow the solidifying plug 5 to remain in the closed can from 24 to 48 hours. At the expiration of that time, the cover would be removed, and any liquid at the top of the solution would be poured off, the plug removed, and then the cavity left by the plug filled with a nitro-cellulose solution corresponding to that originally used, and such an additional quantity poured into the can or container as will bring the top of the solution approximately to the line 7, that is, just under the cover 4, and then the cover 4 would be replaced tightly. Upon standing, the water in the solidified nitro-cellulose would diffuse into the new quantity of unsolidified nitro-cellulose solution added and completely solidify it so that the can or container, when it reaches the customer, would be completely filled with a solid alcohol.

By suitably adjusting the proportions of the depth of the nitro-cellulose solution and the diameter of the cylinder 5, I may very greatly decrease the average distance of any given particle of dissolved nitro-cellulose from the solidifying agent, water, in the body 5, so that although, by the solidifying method by pouring water on the top of the nitro-cellulose solution it is necessary for the water to travel the entire distance from the top to the bottom of the solution in order to completely solidify it, in my method the distance for the water to travel will be so greatly decreased that a much quicker solidification will take place. By suitable proportioning, the rapidity of the solidification may be made almost anything desired, that is, by surrounding the

body 5 with an extremely thin layer of nitro-cellulose solution, solidification will take place almost immediately, but as the layer around the body 5 increases in thickness the solidification will be to that extent more slow. The preferred speed is a solidification by standing over night.

5

The moisture content of the plug or body 5 determines the moisture content of the solidified nitro-cellulose and, although I prefer a moisture content as specified, nevertheless it is to be understood that as the moisture content of the plug or body 5 may be varied, so may the moisture content of the solidified nitro-cellulose, and that moisture content, by reason of the control of the moisture content of the plug or body 5, may be controlled within quite narrow limits. If a liquid collects upon the top of the nitro-cellulose solution upon standing while being solidified, it will consist of water and alcohol. This may be

10

15

20

poured off if desired.

Although I prefer to remove the soap plug and fill the cavity produced thereby with more of the cellulose base nevertheless, I may remove the soap plug and put nothing in its place, or I may leave the plug in place. In case I leave the plug in place, I do not mean to exclude a shortened plug whereby the cellulose nitrate may be placed over the top thereof.

25

Although I have particularly described one particular physical embodiment of my invention, and explained the principle of the operation thereof, nevertheless, I desire to have it understood that the form selected is merely illustrative, but does not exhaust the possible physical embodiments of the idea of means or method underlying my invention.

30

What I claim as new and desire to secure by Letters Patent of the United States, is:

35

1. The method of solidifying a nitro-cellulose solution which consists in placing a solid body of water moist soap therein.
2. The method of solidifying a nitro-cellulose solution which consists in placing therein a solid alcoholic water containing neutral soap.
3. The method of solidifying a nitro-cellulose solution which consists in placing therein a solid body of an alcoholic water containing neutral sodium stearate.
4. The method of solidifying an ethyl alcohol solution of nitro-cellulose, which consists in immersing a solid neutral alcoholic sodium stearate containing water therein.
5. The method of solidifying an ethyl alcohol solution of a cellulose ester, which consists in immersing a solid neutral alcoholic sodium stearate containing water therein.

40

45

50

55

HERBERT KRANICH.